# EUROPEAN PATENT SPECIFICATION

(11) **EP 2 104 764 B1**
(45) Date of publication and mention of the grant of the patent: **27.06.2012**
(21) Application number: 08701235.7
(22) Date of filing: 04.01.2008
(51) Int. Cl.: D07B 1/16, D07B 1/06

(54) **CABLE WITH LOW STRUCTURAL ELONGATION**
KABEL MIT GERINGER STRUKTURELLER DEHNUNG
CÂBLE À FAIBLE ALLONGEMENT STRUCTURAL

(30) Priority: 08.01.2007 EP 07000237
(43) Date of publication of application: 30.09.2009
(73) Proprietor: NV Bekaert SA, 8550 Zwevegem (BE)
(72) Inventor: BRUYNEEL, Paul, B-8710 Ooigem (BE); VANCOMPERNOLLE, Stijn, B-9000 Gent (BE); VANDERBEKEN, Bert, B-8790 Waregem (BE)
(86) International application number: PCT/EP2008/050053
(87) International publication number: WO 2008/084010

(56) References cited:
- EP-A- 0 125 518
- EP-A2- 1 457 596
- WO-A-99/06628
- WO-A-03/044267
- WO-A-2004/076327
- WO-A-2005/043003
- GB-A- 1 069 461
- JP-A- 59 125 988

## Description

### Field of the invention.

The present invention relates to a cable. More specifically present invention relates to a cable with limited elongation.

### Background of the invention.

Cables and more specifically control cables are widely used to transmit movement, such as cable for window elevator system, cables used to open and close braks of scooters, bicycles and other vehicles. In these and many other applications, a limited elongation of the cable is required.

Cables are also widely used as tension member to reinforce polymer materials, such as steel cords to reinforce radial tires, cables to reinforce transmission belts, timing belts or flat hoisting belts. In these applications, a limited elongation of the cable is also required.

Generally, the tensile curve of a cable of prior art takes the form of "hockey stick" curve as illustrated by FIGURE1. At the initial elongation period, the elongation of the cable is large while the tension is low, and the curve is relative flat. At the terminal elongation period, the elongation of cable is almost linear to the tension of the cable as illustrated by line 120 in FIGURE1. The elongation of the cable increases steadily with the increase of the tension. At this stage, the increase of the elongation of the cable is proportional to the increase of the tension of the cable, i.e. Δε=Δδ/E, wherein Δε is the increase of the elongation of the cable, Δδ the increase of the tension of the cable, and E the module of the cable. This is called the elastic elongation. If we extend line 120 to intersect with the abscissa axis, the intersection point ε0 represents the structural elongation at low tensile stresses of the cable. Therefore, the elongation of a cable at certain tensile stress can be expressed by ε=ε0+δ/E. From this equation, we can see that the total elongation of a cable at certain tensile stress comprises two portions of elongations: structural elongation and the elastic elongation. Therefore, there are two approaches to get a cable with limited elongation. One way is to decrease the structural elongation of the cable, and the other way to increase the E module of the cable, because the elongation under tensile decreases when the E module of the cable increases.
Besides, structural elongation ε0 of a cable is unstable and unpredictable, because there are a lot of facts, such as the structure of the cable, the voids between the filaments of the cable, and the pretension of the filaments when cabling the cable, that determine the structural elongation of a cable. Therefore, the unstable and unpredictable behavior of structural elongation of a cable causes problems to predict the total elongation of the cable under tension and more scrap during the start-up of machine producing for instance the high-precision timing belts. Hence, further reducing or almost eliminating the structural elongation ε0 can improve the predictability of the tension-elongation curve of the cable and facilitate the manufacturing process.

WO03044267A1 disclosed a cable with limited elongation, less than 0.05% at a permanent force of 50N, after being subjected to a force of 450N. This improvement is achieved by a cord comprising a steel cord and a polymer material. The low elongation is highly related to the penetration of polymer material into the steel cord, but there are limits on the penetration rate and the pressure for the extrusion process.

WO2005043003A1 disclosed a fine steel cord with low structural elongation. The low structural elongation is achieved by using a special cabling process. This special cabling process not only decreases the productivity of the cabling process but also ask for a lengthy fine tune procedure to set the tension of the filaments or strands.

### Summary of the Invention.

It is an objective of the present invention to eliminate the drawback of the prior art. It is also an objective of the present invention to further limit the elongation of a cable without complicating the manufacturing process of the cabling process.

According to the present invention, a cable is provided comprising a steel cord and a polymer material. The steel filaments of the steel cord are coated with an adhesive before the penetration of the polymer material. The cable has a structural elongation less than 0.025%. Besides, the E module of the cable increases by more than 4% compared with the E module of the bare steel cord. These two Improvements further decrease the total elongation of the cable at certain load. The polymer filling rate is more than 70%. The thickness of the polymer coating is less than 10µm.

The cable as subject of the invention comprises a steel cord, which on its turn comprises several steel filaments.

The tensile strength of the steel filaments for the steel cord are preferably more than 1700N/mm², or more than 2200N/mm² or even more than 2600N/mm², most preferably more than 3000N/mm² or even more than 4000N/mm². The diameter of the filaments is less than 400µm, preferably less than 210µm, most preferably less than 110µm.

All filaments may have an identical diameter. Possible the diameter of the filaments may differ from each other. Preferably, the diameter of the filaments providing an inner strand of the cable is larger than the diameter of the filaments used to provide the outer strands or layer of filaments to the cable, which improves the penetration of the polymer material into the void spaces of the cable.

Steel cords have an inner layer or core, which is preferably a strand of several steel filaments. Around such core, at least one layer of additional steel elements is provided. The steel elements of the additional layer can either be steel filaments or steel strands, on its turn comprising steel filaments. Various steel cord construction may be used.

Examples here are:
- Multi-strand steel cord e.g. of the m x n type, i.e. steel cords, comprising m strands with each n steel filaments, such as 4x7x0.10, 7x7x0.18, 8x7x0.18 or 3x3x0.18; the last number is the diameter of the steel filament expressed in mm;
- Multi-strand steel cord, comprising a core strand of c metal filaments, and m strands of n steel filaments, surrounding the core strand. These steel cords are hereafter referred to as c+mxn type cords, such as 19+9x7 or 19+8x7 cords;
- Warrington-type steel cords;
- Compact cords, e.g. of the 1xn type, i.e. steel cords comprising n steel filaments, n being greater than 8, twisted in only one direction with one single step to a compact cross-section, such as 1x9x0.18; the last number is the diameter of the filament expressed in mm;
- Layered steel cord e.g. of the c+m(+n) type, i.e. steel cord with a core of c filaments, surrounded by a layer of m filaments, and possibly also surrounded by another layer of n filaments, such as 2+4x0.18; the last number is the diameter of the filaments expressed in mm.

The steel composition of the steel cord is preferably a plain carbon steel composition, i.e. it generally comprises a minimum carbon content of 0.40% (e.g. at least 0.60% or at least 0.80%, with a maximum of 1.1%), a manganese content ranging from 0.10 to 0.90% and a silicon content ranging from 0.10 to 0.90%; the sulfur and phosphorous contents are each preferably kept below 0.03%; additional micro-alloying elements such as chromium (up to 0.2 to 0.4%), boron, cobalt, nickel, vanadium...may be added to the composition; stainless steel compositions are, however, not excluded. The production of the steel filaments and the steel cords is performed according to known prior art techniques of wet drawing followed by cabling or bunching.

After an optional cleaning operation, the steel cord is then coated with an adhesive selected from organo functional silanes, organo functional titanates and organo functional zirconates which are known in the art for the improvement of adhesion between the steel cord and polymer material. Preferably, but not exclusively, the organo functional silanes are selected from the compounds of the following formula:

Y-(CH₂)_{N}-SiX₃

Wherein:
Y represents an organo functional group selected from -NH₂, CH₂=CH-, CH₂=C(CH₃)COO-, 2,3-epoxypropoxy, HS- and, Cl-
X represents a silicon functional group selected from -OR, -OC(=O)R', -Cl wherein R and R' are independently selected from C1 to C4 alkyl, preferably -CH3, and -C2H5; and
n is an integer between 0 and 10, preferably from 0 to 3.

Besides the organo functional silanes mentioned above, there are other steel PU adhesives commercially available on the market. They are sold under the name Chemosil (made by the German company Henkel) and Chemlock (made by Lord Corporation).

The polymer material used for the present invention can be any elastomeric material that can conveniently be applied to the steel cord with sufficient adhesion. More preferably a thermoplastic elastomer (TPE) can be used. Non-delimiting examples are polystyrene/elastomer block copolymers, polyurethane (PU) or polyurethane copolymers, polyamide/elastomer block copolymers, thermoplastic vulcanizates. Preferably thermoplastic polyurethane is used. Homopolymers of ester, ether or carbonate polyurethane may be used, as well as copolymers or polymer blends. Preferably, the polymer material has a shore hardness varying between 30A and 90D.

The polymer penetration rate of a cable as subject matter of the present invention Is more than 70%, and preferably more than 90%. The steel cord used to provide a cable as subject matter of the present invention comprises several steel filaments being transformed into a steel cord, using a steel cord construction. Due to the steel cord construction, void spaces are provided between the steel filaments of the steel elements of the cord. Also void spaces are provided between the steel elements. "Void space" as used hereafter is to be understood as all area of a radial cross-section of the cord, located inwards of the imaginary circle which encircles a radial cross section of the steel cord which area is not occupied by steel. Therefore, the polymer penetration rate of a cable of present invention is defined as the ratio in percentage of the void space filled by polymer to the void space which is not occupied by steel.

The thickness of the polymer coating of the present invention is less than 10µm. The optical diameter of the steel cord used to provide a cable as subject matter of the present invention is the diameter of the smallest imaginary circle, which encircles a radial cross section of the steel cord. The optical diameter of the cable of the present invention is the diameter of the smallest imaginary circle, which encircles a radial cross section of the cable. Therefore, the thickness of the polymer is defined as the half of the difference of the optical diameter between the cable and the steel cord.

### Brief description of the drawings.

The invention will now be described into more detail with reference to the accompanying drawings wherein
- FIGURE 1 Is a tensile curve of a cable of prior arts;
- FIGURE 2 is a cross-sectional view of a cable incorporating the present invention;
- FIGURE 3 is a tensile curve of a cable incorporating the present invention.

Item 110 is the tensile curve of a cable of prior arts;
Item 120 is a line representing the E module of a cable of prior arts;
Item 211 is a cable incorporating the present invention;
Item 212 is a steel cord for the cable incorporating the present invention;
Item 213 is a steel filament for the cable incorporating the present invention;
Item 214 is the optical diameter of the steel cord for the cable incorporating the present invention;
Item 215 is a polymer material used for the cable incorporating the present invention;
Item 216 is the optical diameter of the cable incorporating the present invention;
Item 217 is the thickness of the polymer coating of the cable incorporating the present invention;
Item 218 is the void space in the cable incorporating the present invention;
Item 219 is the steel strand for the cable incorporating the present invention;
Item 310 is the tensile curve of a cable incorporating the present invention;
Item 320 is a line representing the E module of a cable incorporating the present invention;
ε0 is the structural elongation of a cable;
F(N) is the force in Newton on the test specimen;
E(%) is the elongation in percentage of the test specimen.

### Description of the preferred embodiments of the invention.

In FIGURE 1, there is shown a tensile curve 110 of a cable of prior art, and line 120 represents the E module of the cable. Line 120 extends and intersects with the abscissa axis at the intersection point _{E}0, representing the structural elongation at low tensile stresses of the cable.

As shown in FIGURE 2, there is a cross section view of a cable incorporating the present invention. The cable 211 comprises a steel cord 212, which on its turn comprises several steel filaments 213. The present embodiment shows a steel cord with "7x7xd" structure having seven strands 219, each strand having seven steel filaments 213 of diameter of d mm. The steel cord has an optical cord diameter 214. The steel cord is coated with a polymer material 215, so providing a cable 211 as subject matter of the present invention with an optical cable diameter 216. The thickness 217 of the polymer coating is half of the difference between optical cord diameter and optical cable diameter. As shown in FIGURE 2, preferably the void space 218 between the different steel filaments 213 is substantially filled with polymer material 215.

In FIGURE 3, there is shown a tensile curve 310 of a cable incorporating the present invention, and line 320 represents the E module of the cable. Line 320 extends and intersects with the abscissa axis at the intersection point ε0, representing the structural elongation at low tensile stresses of the cable.

In the following tables, there are shown comparison tests between the cable with prior art and the cable incorporating the present invention. The test is conducted according to ISO test method ISO RA-30-203 on Zwick-Z020 test machine. When one test is finished, the test machine can automatically provide the following test results and the tensile curve of the test specimen.

### Comparison test 1:

Prior art: 1x3+5x7x0.15 steel cord;
Present invention: 1x3+5x7x0.15 steel cord with adhesive treatment and PU coating.

| | Structural elongation ε0 | E module N/mm² | Elongation at 50 N |
|---|---|---|---|
| Prior art | 0.082% | 168072 | 0.125% |
| Present invention | 0.021% | 184293 | 0.060% |
| Improvements against prior art | - 74% | +9.6% | - 52% |

The test results show that the present invention not only substantially decreases the structural elongation of the cable by 74%, but also further improves the E module of the cable by 9.6%. These two improvements make a substantial progress on the elongation at certain load, the total elongation at 50N decreased by 52%. Besides, the tensile curves in FIGURE 1 and 3 also illustrate this improvement.

### Comparison test 2:

Prior art 1: 7x3x0.15 steel cord;
Prior art 2: 7x3x0.15 steel cord with PU coating;
Present invention: 7x3x0.15 steel cord with adhesive treatment and PU coating.

| | Structural elongation ε0 | E module N/mm² | Elongation at 50 N |
|---|---|---|---|
| Prior art 1 | 0.044% | 176357 | 0.119% |
| Prior art 2 | 0.031% | 180437 | 0.105% |
| Present invention | 0.004% | 182778 | 0.077% |
| Improvements against prior art 1 | -91% | +4% | - 35% |

The test results show that the present invention not only substantially decreases the structural elongation of the cable by 91%, but also further improves the E module of the cable by 4%. These two improvements make a substantial progress on the elongation at certain load, the total elongation at 50N decreased by 35%. Besides, the tensile curves in FIGURE 1 and 3 also illustrate this improvement.

Compared with prior art, the use of an adhesive on the surface of steel filaments before the application of polymer material further improves the anchorage of steel filaments inside polymer material. The steel filaments of the steel cord are constrained from slipping and turning even there are some void spaces unfilled by polymer material, which further limits the structural elongation of the cable. Besides, the improved anchorage of steel filaments inside polymer material also improves the E module of the cable because there is no slippage or peeling between steel filaments and polymer material.

A further improvement to the present invention is characterized by the thickness of the polymer coating of the cable. A cable with polymer coating of 1 0pm only marginally increases the diameter of the cable, which is especially valuable for the cable used as tension member to reinforce synchronous belt. Because the synchronous belt is molded in a semi-open mold where the polymer material is poured into the mold or extruded with a low pressure, the polymer material inside the mold has limited ability to flow between the tension members and to form the final requested shape (toothed, flat, even, ...). Therefore, a fine cable with less than 10µm polymer coating will leave more space for the polymer material to flow inside the mold and to form a flat and even belt.

Another application with this fine cable with less than 10µm polymer coating is for window elevator system. Because the cable used for window elevator system needs to be clamped by metal nipples at the end of the cable to connect other parts, cables with thick polymer coating can not guarantee a secured connection between the end of the cable and the nipple. The nipple clamps on the polymer coating and the polymer coating transfers the tension to the steel cord inside. Since the tensile strength of the polymer material is quite low compared with that of the steel cord, the connection between cable and nipple breaks at low load, and the load transmission ability of the cable is undermined due to this weak point. When a cable with less than 10µm polymer coating is used in a window elevator system, the metal nipple clamps directly to the steel cord because of the deformation of thin coating of polymer material. This application secures the connection between cable and nipple and eliminates the weak point for the system. Besides, when the coating thickness is less than 10µm or even 0µm, from the outside the cable is virtually the same as a bare cable with the same friction and wear properties. This might be of a big advantage when one would like to substitute a bare cable by such a products in a cable system since there is no need to change the guiding part, cable tubes, etc.

Another improvement with present invention is to use the cable as the subject matter of present invention to build a multi-strand rope for hoisting applications such as elevator ropes. Firstly, the elevator industry is looking for ropes with limited elongation. Since the strands have limited elongation, the rope will have a limited elongation either. Hence, elevator ropes using present invention meet this requirement. Secondly, the elevator industry is looking for ropes that are capable of running on small sheave diameters. The standard elevator uses ropes that respect the generally accepted sheave diameter "d" over rope diameter "D" ratio of 40. When traditional all steel ropes are used in conditions where the d/D ratio is lower than 40, the fatigue life of ropes drops significantly. One of the failure causes of the ropes under these conditions is excessive inter-strand and inter-wire fretting. Although a polymer coating on the rope can reduce the fretting and improve the fatigue life of the rope, a thick polymer coating is needed to secure an endurable polymer sheath and the thick coating increase the diameter of the rope. Present invention solves this dilemma. On one hand, steel strands are coated with polymer to reduce the fretting. On the other hand, adhesive treatment improves the connection between steel and polymer and makes a thin coating possible. Therefore, ropes made of cables of present invention are suitable for hoisting applications.

## Claims

1. A cable (211) comprising a twisted steel cord (212), wherein the cable (211) comprises a polymer (215) coating of a polymer (215) material, wherein the steel filaments (213) of said steel cord (212) are coated with an adhesive, the polymer (215) filling rate of said cable (211) being more than 70%, the structural elongation of said cable (211) being less than 0.025%, the E-module of said cable (211) being 4% greater than that of said steel cord (212),
**characterized in that** the thickness of the polymer (215) coating is less than 10 µm or 0 µm.

2. A cable (211) as claimed in claim 1, **characterized in that** the polymer (215) filling rate is more than 90%.

3. A cable (211) as claimed in any one of claim 1 to 2, **characterized in that** said polymer material (215) is a thermoplastic polymer.

4. A cable (211) as claimed in claim 3, **characterized in that** said thermoplastic polymer is polyurethane.

5. A multi-strand rope for hoisting applications comprising more than one cable (211) as claimed in claim 1 to 4.

## Patentansprüche

1. Kabel (211), umfassend einen verdrillten Stahlkord (212), wobei das Kabel (211) einen Polymermantel (215) aus einem Polymermaterial (215) umfasst, wobei die Stahlfilamente (213) des Stahlkords (212) mit einem Haftmittel beschichtet sind, wobei der Polymorfüllgrad (215) des Kabels (211) mehr als 70 % beträgt, wobei die Strukturdehnung des Kabels (211) weniger als 0,025 % beträgt, wobei der E-Modul des Kabels (211) um 4% größer ist als jener des Stahlkords (212),
**dadurch gekennzeichnet, dass** die Dicke des Polymermantels (215) weniger als 10 µm oder 0 µm beträgt.

2. Kabel (211) nach Anspruch 1, **dadurch gekennzeichnet, dass** der Polymerfüllgrad (215) mehr als 90 % beträgt.

3. Kabel (211) nach einem der Ansprüche 1 bis 2, **dadurch gekennzeichnet, dass** das Polymermaterial (215) ein thermoplastisches Polymer ist.

4. Kabel (211) nach Anspruch 3, **dadurch gekennzeichnet, dass** das thermoplastische Polymer Polyurethan Ist.

5. Mehrlltzensell für Hebeanwendungen, umfassend mehr als ein Kabel (211) nach Anspruch 1 bis 4.

## Revendications

1. Câble (211) comprenant une corde d'acier tordue (212), dans lequel le câble (211) comprend un revêtement polymère (215) d'un matériau polymère (215), dans lequel les filaments d'acier (213) de ladite corde d'acier (212) sont revêtus d'un adhésif, le taux de remplissage de polymère (215) dudit câble (211) étant supérieur à 70 %, l'allongement structurel dudit câble (211) étant inférieur à 0,025 %, le module E dudit câble (211) étant supérieur de 4 % celui de ladite corde d'acier (212),
**caractérisé en ce que** l'épaisseur du revêtement polymère (215) est inférieure à une valeur de 10 µm ou vaut 0 µm.

2. Câble (211) selon la revendication 1, **caractérisé en ce que** le taux de remplissage de polymère (215) est supérieur à 90 %.

3. Câble (211) selon l'une quelconque des revendications 1 à 2, **caractérisé en ce que** ledit matériau polymère (215) est un polymère thermoplastique.

4. Câble (211) selon la revendication 3, **caractérisé en ce que** ledit polymère thermoplastique est du polyuréthanne.

5. Cordage multibrins pour des applications de levage comprenant plus d'un câble (211) selon l'une des revendications 1 à 4.
